

June 7, 1938.

W. J. SPARLING

2,119,833

CAST IRON ALLOY AND METHOD OF PRODUCING THE SAME

Filed June 21, 1935

3 Sheets-Sheet 1



Fig.1.



Fig.3.



Fig.5.

FERRITE  
GRAIN  
BOUNDARIES



Fig.6.

SPHEROIDIZED  
CEMENTITE



Fig.8.



Fig.9. Inventor:  
William J. Sparling.  
By Parker & Collings, Inc.

June 7, 1938.

W. J. SPARLING

2,119,833

CAST IRON ALLOY AND METHOD OF PRODUCING THE SAME

Filed June 21, 1935

3 Sheets-Sheet 2

*Fig. 2.*



*Fig. 4.*



*Fig. 7.*



Inventor:  
William J. Sparling,  
by Barker & Collings,  
Atty's.

June 7, 1938.

W. J. SPARLING

2,119,833

CAST IRON ALLOY AND METHOD OF PRODUCING THE SAME

Filed June 21, 1935

3 Sheets-Sheet 3

Fig. 10.



Fig. 11.



WITNESSES  
A. B. Wallace.  
G. L. S. G.

INVENTOR.  
William J. Sparling  
BY  
Barber & Collings  
His ATTORNEYS.

## UNITED STATES PATENT OFFICE

2,119,833

CAST IRON ALLOY AND METHOD OF PRO-  
DUCING THE SAMEWilliam J. Sparling, Milwaukee, Wis., assignor to  
Chain Belt Company, Milwaukee, Wis., a cor-  
poration of Wisconsin

Application June 21, 1935, Serial No. 27,766

7 Claims. (Cl. 148—21.8)

This invention relates to ferrous metal alloys, and more especially to ferrous alloys which include graphitizing accelerating and retarding elements; for example, alloys of iron, carbon, copper and manganese. The invention also comprises a novel heat treatment of castings made from such ferrous metal alloys; and one of its principal objects is to produce a white iron alloy suitable for making white iron castings, which, after being subjected to said heat treatment, will possess higher ductility, higher impact value, higher tensile strength, higher resistance to corrosion, and higher resistance to wear, than have been heretofore obtainable in white iron castings, thereby greatly increasing the durability of such castings in practically every use to which cast iron products are put.

A further object is the improvement of ferrous metal alloys, and more especially ferrous alloys having inclusions of carbon and graphitizing accelerating and retarding elements, for example alloys of iron, carbon, copper, and manganese. The invention has for a further object a novel heat treatment of castings made from such ferrous metal alloys; and its main object is to produce a white iron alloy suitable for making white iron castings, which after being subjected to the novel heat treatment described herein will possess higher ductility, higher resistance to impact forces, a greater tensile strength, higher resistance to corrosion, and higher frictional wear resistance, than have, so far as heretofore known, been obtainable in castings made of white iron; and thereby greatly increasing many of the desirable qualities of such castings.

The said ferrous metal alloys and the heat treatment herein described are inter-related to the extent that if the said alloys are subjected to the said heat treatment, the better results stated above are obtained to a greater degree than if other known heat treatments are employed.

The ferrous metal alloys and the heat treatment of this invention are so inter-related that the desirable qualities heretofore mentioned are attained to a higher degree in castings made of the alloy and heat treated according to the method of this invention, than are secured in castings of the alloy heat treated in a different manner, or in castings of a different composition when heat treated in accordance with the method of this invention.

The term "white cast iron" is applied in the industry to a cast ferrous metal containing appreciable amounts of carbon and silicon, which

elements are so proportioned as to impart to the cast metal, when fractured, a silver-white appearance. The usual white cast iron of commerce also contains some sulphur, phosphorus, and manganese, all in small quantities, and the iron may also contain traces of other elements as impurities which do not have an appreciable effect upon the physical properties of the cast product.

The amounts of carbon and silicon, and their arrangement in the cast metal, are such as to distinguish the iron from steel as generally defined, and are so proportioned as to prevent the separation of the carbon into flake graphite during the cooling or freezing of the cast metal, thereby distinguishing white cast iron from gray cast iron. While such metal as cast is not ductile but very hard and brittle, it may be subjected to a heat-treatment, commonly termed "malleableizing," to develop therein appreciable ductility.

White cast iron for the malleableizing treatment, as heretofore usually made, has a composition approximately within the following limits—

|            | Per cent     | 25 |
|------------|--------------|----|
| Carbon     | 1.90 to 3.00 |    |
| Silicon    | 1.30 to 0.60 |    |
| Phosphorus | 0.08 to 0.16 |    |
| Sulphur    | 0.05 to 0.12 | 30 |
| Manganese  | 0.20 to 0.40 |    |

balance substantially iron. Castings of such composition, when malleableized in the usual American method, are the well known black-heart malleable cast iron products and are characterized by usually having physical qualities approximately within limits as follows—

|                    |                    |                  |
|--------------------|--------------------|------------------|
| Tensile strength   |                    |                  |
|                    | pounds per sq. in. | 45,000 to 60,000 |
| Elastic limit      | do                 | 32,000 to 38,000 |
| Elongation in 2"   | per cent           | 40               |
| Hardness (Brinell) |                    | 25 to 10         |
| Impact value       | foot pounds        | 115 to 140       |

The impact values as herein stated are the average values obtained in numerous tests conducted with a specially constructed impact machine which is similar to the standard Charpy machine, with the exception that my new machine is designed to take rough cast test bars  $\frac{3}{8}$ " sq. by 3" long, while the standard Charpy machine is designed to take machine-finished test bars of smaller size. In my work the test bars were not notched, as required in the standard Charpy test, because notching the surface

45

50

55

of a malleable casting, or a casting made of my special alloy, more appreciably decreases the impact value than would be occasioned on a steel test bar usually used in the Charpy method of determining impact value. However, the specific figures herein shown for impact in foot pounds are representative of the impact value and are comparable to standard Charpy values but not to the same scale because of the size and section of the specimens. The figures for impact are comparable between themselves and give a good indication of the impact value of malleable iron and my alloyed ferrous metal.

The average corrosion resistance of ordinary malleable iron of the above physical properties, as I have determined it, is given in the following table and the figures stated are the average of a great number of tests conducted by me, and show the rate of loss of metal in milligrams per square centimeter of exposed surface of samples during a uniform fixed time period of immersion in the following solutions.

|                               |        |
|-------------------------------|--------|
| 10% salt water solution       | 0.052  |
| 5% sulphuric acid solution    | 23.352 |
| 25% tannic acid solution      | 0.087  |
| 5% lactic acid solution       | 1.190  |
| 5% hydrochloric acid solution | 16.107 |

The malleableizing of white cast iron may be briefly stated as separating by heat-treatment the chemically combined iron and carbon ( $Fe_3C$ ) into iron (ferrite) and finely divided nodules of temper carbon or graphite. To secure the better results of the process, it is essential that substantially all of the carbon be combined chemically with the iron when cast, that is, there should be no free graphitic carbon in the cast metal before practicing the malleableizing process. Another essential is that the silicon, which acts as a graphitizer, be within well defined limits, as is known to those acquainted with the art.

It is well known that certain elements, when combined with iron containing carbon, act as retarders, that is, impede graphitization of the carbon; and that others act as accelerators, that is, promote graphitization, during the malleableizing process. For example, sulphur, manganese and chromium are retarders, while aluminum, nickel, and copper, in small quantities, are accelerators of the phenomena of graphitization. Retarding elements are characterized as forming compounds with molten iron which may be said to act as films that apparently prevent the carbon molecules from migrating together during the malleableizing process, which film formations however, are preventable by appropriate changes in composition of the metal charge before melting. For example, it is well known that sulphur in white iron forms sulphur-iron compounds, apparently having a filming character which prevents graphitization. On the other hand, it is also well known, that sulphur will combine with any manganese in the molten metal in preference to iron, forming small rounded nodules of manganese sulphide which apparently do not interfere with the graphitization process, and therefore it is common practice to have sufficient manganese in the metal to insure the sulphur combining therewith.

The art has heretofore sought a manganese value slightly in excess of twice the sulphur content to act as a "neutralizer," but not in an amount greater than 0.6%, as larger percentages of manganese have tended to make the iron difficult to malleableize, and after the malleableizing

process the metal is apt to be quite hard and deficient in ductility.

Heretofore, in adding copper to iron, it has been customary to also introduce chromium to neutralize the so-called "softening" effect (which for example may be due to graphitizing under certain temperatures) of copper on the product. I have discovered that with an excess of manganese over the normal amount of less than .60%, copper may be introduced into the molten metal in quantities as great as 1.5 percent without adverse effect, and with the use of an excess of manganese, it is not necessary to have chromium in the mixture, as apparently the excess of manganese neutralizes any softening effect (which for example may be due to graphitizing under certain temperatures) the copper may have.

The present invention is a development growing out of the broad invention described and claimed in the co-pending application of Maurice G. Jewett and Samuel C. Harris, Serial No. 564,634, filed September 23, 1931, now Patent 2,008,452, dated July 16, 1935, in that it relates to a heat treated cast iron product in which the major portion of the carbon is in graphitic form, and the cementite is in spheroidized or globular form.

In the present invention, however, by alloying white iron with manganese in an amount above normal practice, and with copper above that heretofore proposed, I am enabled to secure a cast iron product in which, after heat treatment, the spheroidized cementite, instead of being substantially uniformly dispersed throughout the matrix, as in said prior invention, is re-arranged to apparently interlock at the grain-crystal boundaries of the ferrite and thereby make these cleavage planes stronger. It is this re-arrangement of the spheroidized cementite into interlocking relation, with criss-crossing of the ferrite grain-crystal boundaries, to which I ascribe in a large measure the increased impact value of my improved cast ferrous metal alloy, and which arrangement is called herein for short, "net-work structure".

In the accompanying drawings forming a part of this specification:—

Fig. 1 is a copy of a photomicrograph at 1000 diameters of a polished and etched fracture surface of regular white iron of normal analysis, malleableized in the usual manner;

Fig. 2 is a graph of the heat treatment accorded to white iron in the malleableizing process;

Fig. 3 is a copy of a photomicrograph at 1000 diameters of a polished and etched fracture surface of regular white cast iron after heat treatment according to the said Jewett and Harris Patent 2,008,452, above noted; said heat treatment comprising heating to about 1600° F. then immediately quenching, then reheating to about 1325° F. and then again quenching; the illustration exhibiting a spheroidized-pearlitic-sorbitic grain structure;

Fig. 4 is a graph of the heat treatment accorded to the metal shown in Fig. 3;

Figs. 5 and 6 are copies of photomicrographs at 200 diameters and 1000 diameters respectively, of a polished and etched fracture surface of my new alloy, containing 2.29 percent carbon, 0.83 percent silicon, 0.85 percent manganese, and 1.00 percent copper; which alloy has been heated to 1700 degrees F. for thirty hours, then quenched below the critical temperature, then reheated to 1270 degrees F. for thirty hours, then heated to

1340 degrees F. for five hours and quenched. The said alloy thereafter tested as follows:—tensile strength 90,700 pounds, elastic limit 56,300 pounds, and elongation 13.5 percent. Critical 5 temperatures, as defined herein, are temperatures at which retardation occurs in the heating and cooling curves of iron-carbon alloys, and are attributed to chemical and physical rearrangement of the iron and carbon. In alloys of this type, 10 it is commonly defined as the carbon combining temperature. The critical temperature of my metal alloy may range between 1325° F. and 1375° F.

Fig. 7 is a graph of the heat treatment accorded to the metal shown in Figs. 5 and 6, and

Figs. 8 and 9 are copies of photomicrographs at 200 diameters and 1000 diameters respectively, of an etched and polished fracture surface of my new alloy, containing 2.27 percent carbon, 0.89 20 percent silicon, 0.83 percent manganese, and 1.00 percent copper; which alloy has been heated to 1700 degrees F. for thirty hours, then quenched below the critical temperature, then reheated to 1270 degrees F. for thirty hours, then heated to 25 1340 degrees F. for two and one-half hours and thereafter quenched. After such treatment the said alloy tested as follows:—tensile strength 80,000 pounds, elastic limit 55,800 pounds, and elongation 17.0 percent.

30 Fig. 10 is a sketch constituting a diagrammatic representation of the structure shown in Fig. 3. It is representative of the structure of the final product obtained in accordance with the process disclosed in the aforesaid Jewett et al. patent.

35 Fig. 11 is a similar diagrammatic representation of the structure shown in Fig. 9, representing the microstructure of the final product produced in accordance with the present invention. In Figs. 10 and 11 the various constituents have been 40 identified in the drawings.

One method of making my alloy of white iron, copper and manganese, is to pour molten iron having a composition corresponding to regular 45 white iron into a ladle containing ferromanganese in sufficient amount to bring the manganese content of the resulting alloy as high as 0.65 to 1.10 percent. The ladle will also contain copper in small pieces, such as stampings 50 from thin sheets, in an amount sufficient to make the copper content of the alloy between, say 0.50 to 1.50 percent. The resulting white iron—copper—manganese alloy, when made in this 55 manner, will, when cast, have a composition substantially within the following limits—

|              | Percent      |
|--------------|--------------|
| Carbon       | 1.90 to 3.00 |
| Silicon      | 1.30 to 0.60 |
| 60 Manganese | 0.65 to 1.10 |
| Copper       | 0.50 to 1.50 |
| Phosphorus   | 0.08 to 0.16 |
| Sulphur      | 0.05 to 0.12 |

65 After being subjected to the heat-treatment hereinafter described, this new alloy will be a cast iron product having physical characteristics within the following limits—

|                             |                                      |
|-----------------------------|--------------------------------------|
| Tensile strength            |                                      |
| 70                          | pounds per sq. in. 67,500 to 110,000 |
| Elastic limit               |                                      |
|                             | pounds per sq. in. 47,500 to 65,000  |
| Elongation in 2"---percent  | 18 to 12                             |
| Hardness (Brinell)          | 170 to 220                           |
| 75 Impact value—foot pounds | 30 to 15                             |

The average corrosion resistance of my new cast iron product, that is to say the rate of loss of metal in milligrams per square centimeter of exposed surface when tested with the same solutions, for the same length of time and under the same conditions as the malleable iron mentioned hereinbefore, is as follows—

|                               |       |
|-------------------------------|-------|
| 10% salt water solution       | 0.016 |
| 5% sulphuric acid solution    | 2.352 |
| 25% tannic acid solution      | 0.047 |
| 5% lactic acid solution       | 0.075 |
| 5% hydrochloric acid solution | 0.511 |

From a comparison of these physical property tables, it is to be clearly seen that my new cast-ferrous alloy has good ductility, a greater average tensile strength, greater impact value, greater hardness thereby being more resistant to wear, and is more resistant to corrosion than malleable 20 cast iron.

In the present heat-treating process, graphically illustrated in Fig. 7, my iron-copper-manganese alloy, prepared for example as above, may be taken from the mold and cleaned, then placed in a suitable furnace having a reducing 25 atmosphere,—that is to say one which will not remove carbon from the surface of the casting,—and brought to a temperature above the critical, that is to say, from about 1600 degrees F. to about 1800 degrees F. This temperature rise may be 30 at a gradual rate and in the example shown in Fig. 7 covers a period of fifteen hours. The alloy is then held at the predetermined temperature, say 1725 degrees F., for a sufficient time to entirely decompose the massive cementite particles, the carbon migrating and forming finely divided graphite nodules; and after this step of the process is completed the matrix is in the austenitic form. The time required for decomposing the cementite and forming austenite is 35 variable with the section and quantitative analysis of the alloy but will usually run between ten hours and thirty-five hours, after which time the alloy is removed from the furnace and quenched in any suitable medium such as air, water, or oil, and 40 brought to a temperature well below the critical, for example, to a temperature of about 1200 degrees.

After the temperature has been lowered below the critical, the alloy is placed in a suitable furnace which has previously been heated to between 45 say 1250 degrees F. and 1300 degrees F., and preferably to approximately 1270 degrees F. (somewhat below the critical range) and held there for a sufficient time to allow the cementite, 50 which is now in pearlitic form, to become completely spheroidized and uniformly distributed throughout the entire matrix in minute particles. The break-down of the pearlite into ferrite and 55 graphite during this part of the process I believe to be largely prevented by the action of the excess of a retarding element such as manganese.

The structure of the metal at this stage is shown by the diagrammatic representation of Fig. 10, and it will be noted that in this condition the 60 structure corresponds to that obtained in accordance with the process of the aforesaid Jewett et al. patent. After a time sufficient to secure the above noted rearrangement of the cementite particles,—which time-period will vary with the 65 size and shape of the article being treated, but which usually ranges between ten and thirty-five hours,—the temperature is raised to between 1325 degrees F. and say 1360 degrees F. Within this last mentioned temperature range, a rear- 70 75

angement of the spheroidized cementite particles takes place and they appear to migrate and rearrange themselves into a compactly interlocking structure along the ferrite grain-crystal boundaries 5 aries. This is the structure of the final product of the present invention, and it may be understood by reference to the diagrammatic representation of Fig. 11, which clearly shows the concentration of spheroidized cementite in the form of a network, or interlocking, in the ferrite grain boundaries, together with some residual spheroidized cementite throughout the grains, i. e., some spheroidized cementite which has not yet migrated to the grain boundaries. This higher 10 temperature is held for a sufficient time to permit this rearrangement of the globular cementite, which is usually between two and one-half and seven and one-half hours, depending upon the chemical composition, size and shape of the casting, and the tensile strength, hardness, impact value, and other physical properties desired in the product; after which the article is quenched in air, water, oil, or other medium with sufficient 15 rapidity to retain the structure secured at the higher temperature.

The product now has a microstructure as shown in Figs. 5 and 6 or Figs. 8 and 9 wherein the spheroids of cementite, instead of being distributed uniformly throughout the matrix, are 20 collected and interlocked into the grain boundaries of the original ferrite grain-crystals in such manner as to form a network interlocking the grain-crystals and to greatly strengthen the grain-crystal boundary cleavage planes. I believe 25 that the copper contained in my alloy, which is an accelerator, plays a very important part in securing this network structure during the final higher heat treatment, as I have discovered that it requires at least .50 percent copper in the mixture to secure the microstructure shown in Figs. 30 5 and 6 or Figs. 8 and 9. It is my theory that during the final high temperature, the copper, (which is an accelerator), when it is in excess of .50 percent, tends to neutralize the effect the 35 manganese (a retardant), may have on the carbon and permits the carbon-iron spheroidized cementite to be expelled from the ferrite grains into an interlocked, closely woven, network structure along the ferrite grain-crystal boundaries.

When normal white cast iron having no excess manganese and no copper incorporated therein, is given the heat treatment shown in Fig. 7, the 40 microstructure remains substantially the same as shown in Fig. 1, and its physical properties do not differ materially from those of malleable iron produced from normal white iron and subjected to the malleableizing process.

If white cast iron having manganese in excess of the normal practice of less than .60%, that 45 is to say, white iron having at least .70% manganese, and having no copper, is accorded the heat treatment shown in Fig. 7, its microstructure will be substantially the same as shown in Fig. 3. After the heat treatment, this product will have a major portion of the carbon divided out of the 50 mixture as fine particles of graphite; however, because of the manganese being above normal, some of the carbon will be retained in carbon-iron combination (Fe<sub>3</sub>C) and appears in the micro-structure as globular or spheroidized cementite quite uniformly interspersed with no definite arrangement throughout the matrix. The tensile strength and hardness of this high-manganese 55 iron product is greater than that of malleable iron of regular white iron composition; but its

impact value is much lower and may be as low as 5 foot pounds. I ascribe this low impact value to the fact that the uniform distribution of the spheroidized cementite throughout the matrix tends toward a rigid and less mobile grain structure, with the result that the fracture takes place through the weaker planes along the ferrite crystal grain boundaries. The character of the fracture is somewhat influenced by the rapidity of testing. Microscopic examination of fractured 10 pieces of such alloy indicates that when tested slowly in a tensile test, some parts of the fracture are through the ferrite crystal, which type of fracture generally shows good ductility, and elongation may be as high as 15%. A microscopic study of pieces fractured by impact determines that impact fracture is almost wholly along the ferrite grain boundary planes. A fracture of this character quite generally indicates a low impact value.

Photomicrographs of numerous pieces of my new white iron-copper manganese alloy, after being accorded heat treatment as indicated in Fig. 7, that is to say with a quick temperature rise near the end of the heat treatment, show a structure substantially the same as Figs. 5 and 6 or Figs. 8 and 9 in which a major portion of the spheroidized cementite is closely interlocked as a network within the grain crystal boundaries of the ferrite; and the physical properties of the several pieces will vary substantially in direct ratio to the time they were held at the final higher temperature. As to the way the physical properties may be changed by varying the time at which my cast iron alloy is held at the final high temperature of my heat treatment, the following figures are given, which I have taken from data compiled from numerous tests, attention being especially called to the change in impact value:—

| Hours at 1340° F.       | 0      | 1 $\frac{1}{4}$ | 2 $\frac{1}{4}$ | 5      | 7 $\frac{1}{2}$ |
|-------------------------|--------|-----------------|-----------------|--------|-----------------|
| Impact value (ft. lbs.) | 0      | 1 $\frac{1}{4}$ | 2 $\frac{1}{4}$ | 5      | 7 $\frac{1}{2}$ |
| Elongation              | 15     | 17              | 21              | 24     | 27              |
| Tensile strength        | 81,200 | 80,300          | 82,200          | 84,100 | 82,000          |
| Elastic limit           | 57,100 | 57,100          | 58,000          | 57,800 | 58,100          |

A microscopic examination of fractured pieces of my heat treated white iron-copper-manganese alloy which have been tested slowly in a testing machine for tensile strength, indicates that the fracture takes place through the ductile ferrite grain crystals, but as these crystals are surrounded by a network of interlocking spheroids of cementite, which are harder and tougher than the ferrite crystals, the fracture must also pull apart the interlocking spheroids, which, I believe, accounts for the increase in tensile strength.

When the product is tested under impact, a microscopic examination of the fracture indicates that the fracture has taken place almost wholly through the ferrite grain crystals and not along the grain boundary planes. Such a fracture is always indicative of high impact value as it takes considerable force under impact to tear apart the ferrite grain crystals.

If the product is placed in a vise and struck a sharp quick blow with a hammer, it shows a very tough fracture and will withstand considerable impact force before yielding, very much more so than a malleable iron product or other heat treated cast iron product.

After effecting the heat treatment described, my alloy will have physical and corrosion-resistant properties substantially within the range stated herein, and for a cast iron product, an exceptionally high impact value. I ascribe the same

to the network-like structure of spheroidized cementite within the ferrite grain-crystal boundaries, which I believe is attained by my heat treatment of a cast iron alloy having an excess 5 retarder element and an appreciable amount of an accelerator element.

While I have described my invention by reference to certain practical embodiments in order that the same may be used by those skilled in the 10 art, it will be obvious that other embodiments may be made without departing from the principles of the invention, and, accordingly, it will be understood that the scope of my invention is not to be limited except as may be required by the 15 following claims.

I claim—

1. As a new article of manufacture, heat treated white cast iron alloy containing copper from about 0.5 to 1.5 per cent, manganese from 20 about 0.6 to 1.1 per cent, and characterized by containing spheroidized cementite a substantial proportion of which is interlocked in a network structure along the ferrite grain boundaries.

2. As a new article of manufacture, spheroidized white cast iron alloy containing from about 0.65 to about 1.1 per cent of manganese, from about 0.5 to about 1.5 per cent of copper, having spheroidized cementite interlocked in a network along the ferrite grain boundaries, and having a 30 tensile strength of from about 67,500 to about 110,000 pounds per square inch, an elastic limit of from about 47,500 to about 65,000 pounds per square inch, and an impact strength of at least about 15 foot pounds.

3. That method of producing heat treated white cast iron products, comprising heat treating white cast iron containing copper in excess of 0.5 per cent, and manganese in excess of 0.6 per cent, said treatment comprising heating the 40 alloy at temperatures above and below the critical range for times sufficient to produce therein substantially uniformly distributed spheroidized cementite; and further heat treating said iron at a temperature within the critical range of the 45 alloy for a time sufficient to cause said spheroidized cementite in the presence of said copper to migrate to and from an interlocked network structure along the ferrite grain boundaries.

4. That method of producing heat treated

white cast iron products, comprising heat treating white cast iron containing copper from about 0.5 to 1.5 per cent, and manganese from about 0.6 to 1.1 per cent, said heat treatment comprising heating the alloy at from about 1600° to 1800° 5 F. for a time sufficient to decompose massive cementite, quenching to below the critical temperature, reheating to from about 1250° to 1300° F. for a time to form spheroidized cementite; then raising the temperature to 1325° to 1360° F. 10 for a time sufficient to cause said spheroidized cementite to migrate to and form an interlocked network structure along the ferrite grain boundaries.

5. A method of making heat treated white cast 15 iron according to claim 3, the white cast iron alloy containing from about 0.5 to 1.5 per cent of copper, and about 0.6 to 1.1 per cent of manganese.

6. That method of heat treating white cast iron 20 alloys comprising subjecting a white cast iron alloy containing from about 0.5 to 1.5 per cent of copper, and about 0.6 to 1.1 per cent of manganese, to a temperature above the critical temperature for a time sufficient to decompose massive cementite and deposit graphitic carbon; 25 quenching to below the critical temperature; raising the temperature to a point adjacent but below the critical temperature, and maintaining it thereat for a time sufficient to spheroidize cementite substantially uniformly throughout the 30 matrix; then raising the temperature to, and maintaining it within, the critical range, and thereby causing a substantial amount of spheroidized cementite to migrate and interlock in a network structure along the ferrite grain boundaries; 35 and cooling the alloy to preserve said structure.

7. The method of heat treating white cast iron 40 alloys containing from about 0.5 to 1.5 per cent of copper, and about 0.6 to 1.1 per cent of manganese, which comprises heating said alloys to from about 1600° F. to about 1800° F. for a period 45 of time to decompose massive cementite; then quenching to below the critical temperature; reheating to a temperature of from about 1250° F. to about 1300° F. for a period to spheroidize the cementite; then heating in the critical range, from 1325° F. to about 1360° F., for several hours; and then quenching.

WILLIAM J. SPARLING.